

# UNITED STATES PATENT OFFICE.

H. K. SCHAUCK, OF BENVILLE, INDIANA.

## IMPROVED COMPOSITION FOR ROOFING.

Specification forming part of Letters Patent No. **59,462**, dated November 6, 1866.

*To all whom it may concern:*

Be it known that I, H. K. SCHAUCK, of Ben-  
ville, in the county of Jennings and State of  
Indiana, have invented a new and useful Im-  
provement in Composition for Plastic Roofing;  
and I do hereby declare the following to be a  
full and complete description of the ingre-  
dients, with the proportions of each and the  
manner of compounding the same, forming my  
improved plastic roofing composition, suffi-  
cient to enable any person of competent skill  
in the art to make and use my invention.

In the employment of most of the roofing  
compositions the use of tarred paper or some  
other textile substance is required to receive  
the composition and form the complete roof.  
This adds largely to the cost of the covering,  
both in material and labor. The design of my  
improved composition is to be used upon the  
naked sheathing of the roof, or, still more ap-  
propriately, upon a foundation made of narrow  
strips of sufficient thickness, say about one  
inch, nailed to the rafters, as laths are used  
for plastering, with a small space between  
each.

The elements of my improved roofing com-  
position consist of crude coal-tar, common blue  
clay, and flowers of sulphur, in the following  
proportions, to wit: twelve (12) parts dry and  
finely-pulverized blue clay, one (1) part flowers  
of sulphur, mixed and incorporated with a suf-  
ficient quantity of common crude coal-tar to  
form a plastic mass of convenient consistency  
to be handled and applied to the roof with an

ordinary trowel. The clay and the sulphur  
are first mixed in the proportions above stated,  
and then moistened with the coal-tar and  
thoroughly incorporated therewith, enough of  
the latter being used to give to the whole the  
proper consistency, as above stated. All the  
operations of mixing and using the composi-  
tion may be performed while the materials are  
in the cold state, or at a temperature not much  
above 100°. In no case should the tar or the  
composition be boiled.

The composition may be applied to the roof  
with an ordinary trowel, or any convenient  
tool, after the manner of applying plastering.  
The substance will, in a very short time, harden,  
so that it can be walked upon. At the same  
time it will retain sufficient plasticity to ac-  
commodate the ordinary vibrations to which  
roofs are exposed without cracking. It will  
not become fluid from the heat of the sun and  
run, nor will it shrink and crack.

Having fully described my improved roofing  
composition, what I claim as my invention,  
and desire to secure by Letters Patent of the  
United States, is the following:

A roofing composition composed of the sub-  
stances herein specified, in the proportions  
and compounded in the manner substantially  
as described.

H. K. SCHAUCK.

Witnesses:

IRA S. DRAKE,  
JACOB S. DRAKE.